

# United States Patent Office

2,927,873

Patented Mar. 8, 1960

1

2,927,873

## METHOD OF INCREASING THE RESISTANCE OF METALS TO CORROSION

Erik Birger Bengtsson and Olof Ingvar Olsson, Karlskoga, Sweden, assignors to Aktiebolaget Bofors, Bofors, Sweden, a Swedish corporation

No Drawing. Application October 28, 1952  
Serial No. 317,362

Claims priority, application Sweden March 26, 1952

4 Claims. (Cl. 148—6.15)

In such chemical industry where corroding agents are used, the choice of construction material for reaction vessels will often cause great difficulties. The different brands of acidproof steel still do not satisfy all the requirements on resistance to acids, such as nitric acid and sulphuric acid. In particular in such reaction vessels made of acidproof steel, where the reaction occurs at high temperature, the corrosion is considerable in the presence of the above mentioned acids.

This invention relates to a method according to which the resistance of metals to corrosion is increased. By treating the metal with nitric acid, nitrates and/or nitrous gases in the presence of inorganic metal phosphates and/or organic phosphates at elevated temperature and/or under pressure, an increased resistance to the above mentioned corrosive attack is obtained.

In the following some examples are given of the method according to the invention and some figures of results achieved. What henceforward below will be said is however not intended to limit the extent of this invention.

### Example 1

Acidproof steel of type SS3MM (17% Cr, 9% Ni) was immersed in an autoclave, charged with p-nitrotoluene (104 g.), 65% nitric acid (189 g.), water (221 g.) and trisodium ortho phosphate (60 g.). The content of the autoclave was heated, while agitated, to about 190° C., when the oxidation reaction started. The temperature was kept at 185–195° C. for about 20 minutes. The pressure rose thereby to a maximum of 35 kg./cm.<sup>2</sup>. The charge was allowed to cool and after three hours the autoclave was discharged. p-Nitro benzoic acid was formed during the reaction.

The acidproof steel sample had lost some weight but when submitted anew to a similar process (without the presence of phosphate) no loss in weight was found. Simultaneously immersed untreated samples for comparison had suffered a corrosion of 1.2 g./m.<sup>2</sup>/h. When phosphate was present in the latter oxidation a slight gain, in weight by the steel samples was noticed. It has been found that metal plates, once treated in presence of phosphate according to the above, can be exposed to the action of diluted nitric acid at high temperature and high pressure during a long period of time, without being attacked by corrosion. Furthermore it has been found that metals treated in this way are resistant to sulphuric acid, according to Example 2.

### Example 2

Acidproof metal plates, treated according to Example 1, were immersed into 10% sulphuric acid, which was refluxed for 50 hrs. After this time a loss of weight of only 0.1 g./m.<sup>2</sup>/h. could be detected. Even to 50% sulphuric acid the resistance was good. Untreated plates of the same material were submitted to the same acid solutions. These plates were rapidly attacked by the acid with the evolution of hydrogen.

2

### Example 3

Acidproof metal plates treated according to Example 1, were immersed into 80% acetic acid and boiled in this acid for 24 hrs. The loss in weight was after this treatment 0.01 g./m.<sup>2</sup>/h. Under the same conditions untreated plates lost 4 g./m.<sup>2</sup>/h.

### Example 4

Plates of the same steel brand as above were put into an autoclave together with diluted nitric acid and a phosphate of  $\beta$ -picoline. The oxidation of the  $\beta$ -picoline was carried out without mechanical stirring at 220–230° C. and at a pressure of about 40 kg./cm.<sup>2</sup> for one hour. By the oxidation nicotinic acid is formed amongst other products. Plates treated in this way showed the same resistance towards nitric, sulphuric and acetic acid as those described in Examples 1 and 2.

### Example 5

20 In the oxidation of a mixture of pyridine bases with nitric acid at a pressure of 30 kg./cm.<sup>2</sup> and about 200° C., a 33% nitric acid used containing 0.5% ortho phosphoric acid. Acidproof steel samples suffered hereby no loss in weight, but gained slowly in weight.

25 The test plates in the above mentioned experiments were primarily of acidproof steel of different composition. In all the cases the final result has been in agreement with what has been stated in the above related examples.

30 We claim:

1. Method of enhancing the corrosion resistance of acidproof steel which comprises subjecting said steel to the action of dilute nitric acid, the concentration of the acid being about 33%, in the presence of a member of the group consisting of a salt of phosphoric acid and phosphoric acid at a temperature above 185° C. and at a pressure within the approximate range of from 3° to 40 kg. per square cm.
2. Method of enhancing the corrosion resistance of acidproof steel which comprises subjecting said steel to the action of a dilute solution of nitric acid in the presence of a member of the group consisting of a salt of phosphoric acid and phosphoric acid at a temperature above 185° C. and under super-atmospheric pressure.
3. Method of enhancing the corrosion resistance of acidproof steel which comprises subjecting said steel to the action of dilute nitric acid in the presence of a small amount of phosphoric acid at temperatures above 185° C. and under super-atmospheric pressure.
4. Method of enhancing the corrosion resistance of acidproof steel which comprises subjecting said steel to the action of dilute nitric acid in the presence of an alkali metal phosphate at temperatures above 185° C. and under super-atmospheric pressure.

### References Cited in the file of this patent

#### UNITED STATES PATENTS

|    |           |                 |               |
|----|-----------|-----------------|---------------|
| 60 | 1,303,627 | Baines          | May 13, 1919  |
|    | 1,446,016 | Kolsky          | Feb. 20, 1923 |
|    | 1,949,090 | Tanner et al.   | Feb. 27, 1934 |
|    | 2,001,754 | Thompson et al. | May 21, 1935  |
|    | 2,132,511 | Henrich et al.  | Oct. 11, 1938 |
| 65 | 2,283,170 | Batcheller      | May 19, 1942  |
|    | 2,293,716 | Darsey          | Aug. 25, 1942 |
|    | 2,396,457 | Cislak et al.   | Mar. 12, 1946 |
|    | 2,446,060 | Pray et al.     | July 27, 1948 |
|    | 2,694,001 | Hayes et al.    | Nov. 9, 1954  |

#### FOREIGN PATENTS

419,212 Italy Mar. 17, 1947

UNITED STATES PATENT OFFICE  
CERTIFICATE OF CORRECTION

Patent No. 2,927,873

March 8, 1960

Erik Birger Bengtsson et al.

It is hereby certified that error appears in the printed specification of the above numbered patent requiring correction and that the said Letters Patent should read as corrected below.

Column 2, line 37, for "within the approximate range of from 30" read -- within the approximate range of from 30 --.

Signed and sealed this 20th day of September 1960.

(SEAL)

Attest:

KARL H. AXLINE  
Attesting Officer

ROBERT C. WATSON  
Commissioner of Patents